

## UNITED STATES PATENT OFFICE

2,058,085

## SIZING PAPER

Otto Kress and Charles E. Johnson, Appleton, Wis., assignors to The Institute of Paper Chemistry, Appleton, Wis., a corporation of Wisconsin

No Drawing. Application January 28, 1935,  
Serial No. 3,807

17 Claims. (Cl. 92—21)

Our invention relates to the sizing of paper and relates more particularly to sizing with paraffin and the like to produce a paper which is suitable for writing, printing, and the like.

5 We are aware that paraffin has heretofore been suggested in connection with the sizing of paper and especially in admixture with rosin size. However, when such previously-known sizes are set through the use of acidic material, such as alum, 10 the particles of paraffin tend to coalesce to form large aggregates which appear in the finished sheets as translucent or semi-translucent "wax spots" and which also offer trouble in the paper-making operation by forming paraffin spots on 15 the wire, thus interfering with the operation of the paper machine. While this difficulty may be reduced by the use of very small quantities of paraffin, such procedure eliminates the advantage of sizing with paraffin which may be obtained 20 when larger quantities are used.

An object of our invention is to devise a method whereby large quantities of paraffin may be used for sizing while avoiding the disadvantages above referred to.

25 Another object of our invention is to provide, as a new composition of matter, a highly stable emulsion of paraffin or the like suitable for sizing.

We have found that paraffin may be placed in a stable, finely-divided form suitable for sizing 30 by emulsifying it with an emulsifying agent such as a soluble soap, the emulsion being stabilized by a protein material such as, for example, milk casein or soy bean casein. Such an emulsion is highly stable even though the paraffin may be 35 present in quantities up to 75 per cent or more of the solids present in the mixture; the paraffin will not agglomerate upon heating or as a result of the hydrolytic action of water, the action of alkaline-earth fillers, or any other agents commonly used in paper making.

40 According to our invention, the emulsion is broken by addition of an acidic substance, such as alum, resulting in setting the paraffin on the fiber in finely-divided form, each particle being 45 surrounded by a film of protein material.

While we do not wish to limit ourselves to any particular theory of reaction, we believe that the protein which is present in the emulsion, when said emulsion is set by addition of acidic material, surrounds in a molecular film the minute 50 particles of paraffin, thus preventing coalescence thereof into larger particles. We have noted, also, that a mixture of paraffin emulsion and alkaline earth filler, wherein the emulsion has been 55 broken by alum, does not show the presence of a

paraffin film or of particles of paraffin which is visible to the naked eye, even upon boiling and subsequent cooling. Our tests indicate that the paraffin is deposited on the fiber in sub-microscopic particles coated with protein, whereby said particles cannot agglomerate and are not readily removable from the fiber.

## Example

This example is given as merely illustrative of 10 our invention and not as limiting.

The following is a preferred way in which we 15 prepare the paraffin emulsion. Ten parts by weight of soy bean protein are treated with 0.7 part of sodium carbonate by heating to 60° C. under mild agitation with 60 parts of water. To 20 this are added five parts of ammonium oleate for other suitable emulsifying agent, such as turkey red oil, gums like gum arabic, sodium stearate, etc. To this mixture, 40 parts of molten paraffin 25 are slowly run in under agitation. The paraffin which we have been using represents normal paraffin of a melting point of 124° F. but higher melting point paraffin might be used or lower melting point paraffin, even down to ordinary oils. 30 The mixture of casein, emulsifier, and paraffin is stirred with a high speed stirrer or other suitable equipment. The time of mixing is usually approximately 15 minutes, the mixture then being 35 diluted with about 1000 parts of water at approximately 60° C. These temperatures can be adjusted, depending upon the melting point of the paraffin used. The emulsion can likewise be made through the use of a colloid mill or other suitable equipment.

The preferred way in which this casein-paraffin 40 size is used is to add it to the pulp in the beater, and then set the size through the use of alum in the usual manner to give an acidity of from about pH 4.5 to 6.0. After about five minutes, which 45 will ordinarily be sufficient time for the setting of the size, the calcium carbonate or other alkaline earth filler may be introduced in slurry form at a concentration of about two pounds per gallon, if such filler is desired. The usual treatments which are given to pulp in the beater, such as coloring or the possible addition of starch, may also be practiced, if desired. In case it is desired to use some rosin size in conjunction with the special casein-paraffin size, then both types of 50 size may be added to the pulp and set with alum in the usual manner.

In using the special casein-paraffin size along with an alkaline-earth filler, in which case the white waters will be alkaline, the beaters should 55

be made up with fresh water at the normal concentration of beater stock, say, from 4 to 6 per cent. However, the diluting water for the dropping of the beaters may be white water if it is available, and thickened stock such as might be recovered from the usual white water systems may be added just prior to dropping. In case no filler is used or in case any fillers other than alkaline-earth fillers are used, such as ordinary clay, 5 no precautions need be taken with regard to the use of white water, and it may be used to make up the beaters or may be omitted as desired. Wet and dry broke should be handled separately in a broke beater and proportionately dropped to the beater chest, or it may be added in slush form to the beater after the sizing operation.

A typical example for the production of book paper would be about as follows:

|                        | Pounds |
|------------------------|--------|
| 20 Bleached soda pulp  | 500    |
| Bleached sulphite pulp | 500    |

To this pulp is added about 5 per cent by dry weight of the casein-paraffin size, which is then set with alum, as described. To this mixture may be added 300 pounds of alkaline-earth filler, the whole beater having been made up with fresh water but using any excess white water which may be available during the operation of dropping the beater.

The stock from the beater is handled in the usual manner over the paper machine. The mix will be on the alkaline side, in view of the excess of alkaline earth filler, with a pH higher than 35 7.0, and the sizing in the finished sheet will have been accomplished entirely through the use of paraffin in such a finely divided state that there will be no danger of having paraffin spots in the finished paper or of operating troubles resulting 40 from paraffin spots on the wire of the paper machine.

It will be understood that other acid-reacting materials may be used to set the size, although alum is preferred. Also, while we have described 45 the use of alkaline filler, it is understood that our invention is not restricted to this feature—various other types of filler may be used, if desired.

Various modifications and variations coming 50 within the spirit of our invention will doubtless suggest themselves to those skilled in the art. Hence, we do not wish to be limited to the specific embodiments and details herein disclosed except to the extent indicated by the appended 55 claims, which are to be interpreted as broadly as the state of the art will permit.

The term "casein" as used in the claims includes both milk casein and soya bean casein.

We claim as our invention:

60 1. The method of sizing paper comprising introducing into a furnish an aqueous colloidal dispersion of waxy material stabilized with an acid precipitable water-insoluble protein, the latter being present in such a quantity relative to the 65 waxy material that particles thereof deposited on the paper fiber of the furnish are surrounded by a protein film preventing agglomeration of the waxy particles, and adding to the furnish acidic material to precipitate the waxy and protein particles on the fiber with the protein material coating the waxy particles.

70 2. The method of sizing paper comprising introducing into a furnish an aqueous colloidal dispersion of waxy material stabilized with an alkali soluble water-insoluble protein precipitable from

an alkali solution by an acidic material, said protein being present in such a quantity relative to the waxy material that the particles thereof deposited on the paper fiber of the furnish are surrounded by a protein film preventing agglomeration of the waxy particles, and adding to the furnish acidic material to precipitate the waxy and protein particles on the fiber with the protein material coating the waxy particles.

75 3. The method of sizing paper comprising introducing into a furnish an aqueous colloidal dispersion of waxy material stabilized with an acid precipitable water-insoluble protein, the latter being present in such a quantity relative to the waxy material that particles thereof deposited on the paper fiber of the furnish are surrounded by a protein film preventing agglomeration of the waxy particles, and adding to the furnish alum to precipitate the waxy and protein particles on the fiber with the protein material coating the waxy particles.

4. The method of sizing paper comprising introducing into a furnish an aqueous colloidal dispersion of waxy material stabilized with an alkali soluble water-insoluble protein precipitable from an alkali solution by an acidic material, said protein being present in such a quantity relative to the waxy material that the particles thereof deposited on the paper fiber of the furnish are surrounded by a protein film preventing agglomeration of the waxy particles, and adding to the furnish alum to precipitate the waxy and protein particles on the fiber with the protein material coating the waxy particles.

5. The method of sizing paper comprising introducing into a furnish an aqueous colloidal dispersion of waxy material stabilized with an acid precipitable water-insoluble protein, the latter being present in such a quantity relative to the waxy material that particles thereof deposited on the paper fiber of the furnish are surrounded by a protein film preventing agglomeration of the waxy particles, adding to the furnish acidic material to precipitate the waxy and protein particles on the fiber with the protein material coating the waxy particles, and then adding to the furnish an alkaline earth filler.

6. The method of sizing paper comprising introducing into a furnish an aqueous colloidal dispersion of waxy material stabilized with an alkali soluble water-insoluble protein precipitable from an alkali solution by an acidic material, said protein being present in such a quantity relative to the waxy material that the particles thereof deposited on the paper fiber of the furnish are surrounded by a protein film preventing agglomeration of the waxy particles, adding to the furnish acidic material to precipitate the waxy and protein particles on the fiber with the protein material coating the waxy particles, and then adding to the furnish an alkaline earth filler.

7. The method of sizing paper comprising introducing into a furnish an aqueous colloidal dispersion of waxy material stabilized with an acid precipitable water-insoluble protein, the latter being present in such a quantity relative to the waxy material that particles thereof deposited on the paper fiber of the furnish are surrounded by a protein film preventing agglomeration of the waxy particles, adding to the furnish alum to precipitate the waxy and protein particles on the fiber with the protein material coating the waxy particles, and then adding to the furnish an alkaline earth filler.

8. The method of sizing paper comprising introducing into a furnish an aqueous colloidal dispersion of waxy material stabilized with an alkali soluble water-insoluble protein precipitable from an alkali solution by an acidic material, said protein being present in such a quantity relative to the waxy material that the particles thereof deposited on the paper fiber of the furnish are surrounded by a protein film preventing agglomeration of the waxy particles, adding to the furnish alum to precipitate the waxy and protein particles on the fiber with the protein material coating the waxy particles, and then adding to the furnish an alkaline earth 15 filler.

9. The method of sizing paper comprising providing a furnish having present an aqueous colloidal dispersion of a mixture of rosin size and waxy material, the latter being stabilized with an acid precipitable water-insoluble protein, the latter being present in such a quantity relative to the waxy material that particles thereof deposited on the paper fiber of the furnish are surrounded by a protein film preventing agglomeration of the waxy particles, and adding to the furnish acidic material to precipitate the waxy and protein particles on the fiber with the protein material coating the waxy particles.

10. The method of sizing paper comprising providing a furnish having present an aqueous colloidal dispersion of a mixture of rosin size and waxy material, the latter being stabilized with an alkali soluble water-insoluble protein precipitable from an alkali solution by an acidic material, said protein being present in such a quantity relative to the waxy material that particles thereof deposited on the paper fiber of the furnish are surrounded by a protein film preventing agglomeration of the waxy particles, and adding to the furnish acidic material to precipitate the waxy and protein particles on the fiber with the protein material coating the waxy particles.

11. The method of sizing paper comprising providing a furnish having present an aqueous colloidal dispersion of a mixture of rosin size and waxy material, the latter being stabilized with an acid precipitable water-insoluble protein, the latter being present in such a quantity relative to the waxy material that particles thereof deposited on the paper fiber of the furnish are surrounded by a protein film preventing agglomeration of the waxy particles, and adding to the furnish alum to precipitate the waxy and protein particles on the fiber with the protein material coating the waxy particles.

12. The method of sizing paper comprising providing a furnish having present an aqueous colloidal dispersion of a mixture of rosin size and waxy material, the latter being stabilized with an alkali soluble water-insoluble protein precipitable from an alkali solution by an acidic material, said protein being present in such a quantity relative to the waxy material that particles thereof deposited on the paper fiber of the furnish are surrounded by a protein film preventing agglomeration of the waxy particles, and adding to the furnish alum to precipitate the waxy and protein particles on the fiber with the protein material coating the waxy particles.

13. The method of sizing paper comprising providing a furnish having present an aqueous col-

oidal dispersion of a mixture of rosin size and waxy material, the latter being stabilized with an acid precipitable water-insoluble protein, the latter being present in such a quantity relative to the waxy material that particles thereof deposited on the paper fiber of the furnish are surrounded by a protein film preventing agglomeration of the waxy particles, adding to the furnish acidic material to precipitate the waxy and protein particles on the fiber with the protein material coating the waxy particles, and adding to the so-treated furnish an alkaline earth filler.

14. The method of sizing paper comprising providing a furnish having present an aqueous colloidal dispersion of a mixture of rosin size and waxy material, the latter being stabilized with an alkali soluble water-insoluble protein precipitable from an alkali solution by an acidic material, said protein being present in such a quantity relative to the waxy material that particles thereof deposited on the paper fiber of the furnish are surrounded by a protein film preventing agglomeration of the waxy particles, adding to the furnish acidic material to precipitate the waxy and protein particles on the fiber with the protein material coating the waxy particles, and adding to the so-treated furnish an alkaline earth filler.

15. The method of sizing paper comprising providing a furnish having present an aqueous colloidal dispersion of a mixture of rosin size and waxy material, the latter being stabilized with an acid precipitable water-insoluble protein, the latter being present in such a quantity relative to the waxy material that particles thereof deposited on the paper fiber of the furnish are surrounded by a protein film preventing agglomeration of the waxy particles, adding to the furnish alum to precipitate the waxy and protein particles on the fiber with the protein material coating the waxy particles, and adding to the so-treated furnish an alkaline earth filler.

16. The method of sizing paper comprising providing a furnish having present an aqueous colloidal dispersion of a mixture of rosin size and waxy material, the latter being stabilized with an alkali soluble water-insoluble protein precipitable from an alkali solution by an acidic material, said protein being present in such a quantity relative to the waxy material that particles thereof deposited on the paper fiber of the furnish are surrounded by a protein film preventing agglomeration of the waxy particles, adding to the furnish alum to precipitate the waxy and protein particles in the fiber with the protein material coating the waxy particles, and adding to the so-treated furnish an alkaline earth filler.

17. The method of sizing paper comprising introducing into a furnish an aqueous colloidal dispersion of a waxy material stabilized with a protein selected from the group consisting of milk casein and soya bean casein, said protein being present in such a quantity relative to the waxy material that particles thereof deposited on the paper fiber of the furnish is surrounded by a protein film preventing agglomeration of the waxy particles, and adding to the furnish acidic material to precipitate the wax and protein particles on the fiber with the protein material coating the waxy particles.

OTTO KRESS.  
CHARLES E. JOHNSON.